

casing 8 is dropped over the ingot, the ingot, casing and all are raised by the hoist 5, and the molten metal is permitted to solidify.

Forming the entire coating in bath 3 has the advantage of requiring only one bath of molten metal. However, it appears that after repeated dipping of iron ingots, segregating casings, etc. into baths of supermolten metal, the molten copper contains more iron than before—doubtless the result of solution of the iron to a slight extent by the molten copper. This tendency to dissolve the iron is greater, the hotter the molten metal; therefore when extreme purity of the coating is desired, as when making coated ingots to be formed into electrical conductors, it is better to form the coating in two operations, the molten copper at ordinary casting temperature in bath 4 having little or no tendency to dissolve iron.

It is exceedingly important to prevent oxidation of the molten metal, as it is very important that the quality of the metal of the coating shall be good; and it is exceedingly difficult to keep copper and most other metals in a molten condition, and particularly in a supermolten condition, for a long period of time, without serious absorption of oxygen and other gases. I therefore provide covers 19 for both baths which are removed only when and so long as absolutely necessary, and I further cover the surface of the molten metal so far as possible with powdered charcoal, providing a clear space for the passage of the ingot and casing by means of a ring 20 of carborundum or other suitable refractory material which floats on the surface of the molten metal; ring 20 confining the powdered charcoal. I further introduce into the molten metal, from time to time, suitable quantities of a reducing material, such as a compound of silicon with copper or other suitable metal; the silicon of such compound combining with the oxygen of any metallic oxids present or with the oxygen of any GO or CO<sub>2</sub> contained in the molten metal.

Instead of filling the casing 8 from the bottom, as above described, I may cause it to fill with molten metal introduced near the top of the casing. In such case I use a casing such as shown in Fig. 3, having pouring holes 21 in its sides, and a shield 22 normally covering such openings. The bottom plate 12 having been applied to such a casing, with the ingot 7 therein, and the chamber being filled with a non-oxidizing atmosphere, as above described, the chamber is lowered into the molten metal until the openings 21 are submerged; and shield 22 being then raised (or if preferred said shield may be raised just before openings 21 near the surface of the molten metal) the molten metal flows through said openings 21 into the casing, displacing the non-oxidizing atmosphere therein and filling the space between the ingot and the sides of the casing. This method of filling the casing avoids drawing of air into the casing with the inflowing metal (as might be the case if molten metal were poured through a runner into openings 21 without submerging said openings in molten metal) and has the important advantage that the metal which fills the casing may be taken from the very best part of the metal in the bath.

The top layer of molten metal is apt to be poor, owing to the presence of oxids, absorbed gas, etc., and the metal at the bottom of the bath is often bad also; but

the metal intermediate these extremes will be good, if proper care be observed, and if the casing be submerged until the openings 21 are at the level of the good metal, the formation of a coating of good quality is assured. There being no air whatever in the casing during the pouring in this manner, of course there can be no oxidation of the molten metal after it enters the casing, nor any oxidation of the film coating.

Forming a tight joint between the casing and the bottom plate has proved to be a difficult matter, when the coating of ingots of considerable length is attempted. When the ingots treated are relatively short—twelve inches or so—no particular difficulty is experienced in keeping a tight joint between the bottom plate and casing; but when this length is doubled or more, difficulty is experienced. Such difficulty I have overcome by the peculiar construction of bottom plate and lower end of casing, shown in Fig. 2, and by the use of proper packing material. The V-section recess 15 at the lower edge of the casing and the V-section rib 14 of the bottom plate coact to center the casing accurately as it seats on the bottom plate; also since the packing material in recess 15 is in a recess, it is not washed away by the molten metal as the casing descends, but remains in said recess until the rib 14, entering the recess, squeezes out excess of packing material. The casing carries such amount of weight as is necessary to press it tightly against the bottom plate and insure a good joint. For packing material in recess 15 I commonly use asbestos cord or rope, 23, covered with a layer of graphite paste; 24. To protect the casing and bottom plate from the molten metal I also cover them with a layer of graphite wash.

To relieve the pressure on the joint between the casing and bottom plate while raising the filled casing from the molten metal, I may apply vacuum to the casing through valve 10. Likewise, to prevent the formation of bubbles, blow-holes and the like in the metal cast as shown in Fig. 3, I may apply vacuum to the casing during or prior to the entry of the molten metal; whereby gas otherwise entrained in the metal will be drawn off.

By the apparatus above described I can inseparably unite iron and steel with such unlike metals as copper, silver, aluminium, gold, platinum, aluminium bronze, nickel, and cobalt. By film-coating in the first instance with a metal which does not volatilize before reaching the supermolten temperature required (for example, by film-coating with supermolten copper or silver) I can also unite iron and steel with brass and tin bronzes, the zinc or tin of which volatilize or oxidize below the supermolten temperature required to unite them directly to the iron or steel. I can also unite inseparably non-ferrous couples, of the above metals and similar metals, such as copper and silver, for example.

It will be seen that the apparatus is particularly suitable for coating with easily-oxidizable metals, such as nickel, for the coating is entirely protected from contact with the air until cold.

By "producer gas" referred to above, I mean gas made from anthracite, coke, charcoal etc., and containing practically none of the hydrocarbons which tend to "split" or decompose; in other words, I mean an absolutely "fixed" gas.

No. 861,221.

PATENTED JULY 23, 1907.

W. M. MCKENZIE.

NUT TAP.

APPLICATION FILED MAY 23, 1906.



WITNESSES:

*W. T. Daye.*  
Alfred T. Gage

INVENTOR

William M. McKenzie.

BY *E. B. Stockling*

Attorney